

## UNITED STATES PATENT OFFICE

2,080,088

METHOD OF LOWERING POUR POINTS OF  
MINERAL OILSFranz Rudolf Moser, Amsterdam, Netherlands,  
assignor to Shell Development Company, San  
Francisco, Calif., a corporation of DelawareNo Drawing. Application October 25, 1933, Serial  
No. 695,161. In the Netherlands November 2,  
1932

## 13 Claims.

(Cl. 196—1)

The invention relates to a process for reducing pour points of hydrocarbon oils, particularly of lubricating oils.

It has been found that the pour point of viscous hydrocarbon oils can be lowered by adding polymerized Edeleanu extracts and similar extracts of mineral oils. By polymerized Edeleanu extracts and the like are meant Edeleanu extracts or other extracts rich in non-paraffinic hydrocarbons obtained by extraction of mineral oils with solvents, such as furfural, phenol, nitrobenzene, BB'dichloroethyl ether (chlorex), etc., which extracts have been cracked or exposed to heating in the presence or absence of catalysts and have thereby acquired pour point-reducing properties. Such activated or polymerized extracts were found to be far more effective as pour point-reducers, or as sources of pour point-reducing substances, derived in the manner hereinafter disclosed, than any other cracked oils, tars, residues or pitches. In principle, any extract can be used, but as a rule extracts of lubricating oils are to be preferred in view of their better yield of polymerization products.

In the application of polymerized extracts for lowering the pour points of lubricating oils, which, for example, have high pour points by reason of their high paraffin wax contents, difficulties are often encountered due to the fact that these extracts do not dissolve readily in the oil and sometimes have an unfavourable effect on the colour of the lubricating oils.

It has now been found that these drawbacks do not occur when the components of the darkest colour and least soluble in hydrocarbons poor in aromatics are first separated from the polymerization product by means of precipitating agents in which these components are insoluble.

A highly suitable precipitating agent is a kerosene poor in aromatics, while lighter distillates, such as straight run gasoline poor in aromatics, may also be used, as well as a lubricating oil poor in aromatics. Many other liquids are also suitable for precipitation of undesirable dark-coloured substances, such as mixtures of alcohol and ether, ethyl acetate and amyl alcohol.

In some cases the use of a lubricating oil poor in aromatics as precipitating agent may have its advantages. For example, when kerosene or a lighter distillate is used as precipitating agent the resulting dilute oil solution usually has to be concentrated by distillation (with steam or under vacuum, if desired) and the resultant residue applied, as such or dissolved in oil, as a

pour point-reducing agent; however, when a lubricating oil poor in aromatics is used as the precipitating agent the resulting oil solution can be added directly to the oil whose pour point is to be reduced. The effective quantity to be used in each case can be readily ascertained by tests.

In many cases it may be considered preferable to add the polymerized Edeleanu extract treated in the above manner in the form of a solution, so as to facilitate dosing. For instance, if the pour point of a lubricating oil has to be reduced, then a similar lubricating oil may also be used as a solvent for diluting the polymerized extract freed of the undesirable dark coloured substances.

By choosing the right precipitating agent and by regulating its quantity and the treating temperature, it may be assured that substantially only undesirable components are removed from the oil, i. e. those which are least soluble and darkest in colour. These undesirable components, which are removed in the described manner, may be referred to as an asphaltene fraction. Therefore, it is the least soluble and darkest coloured asphaltenes that are removed from the polymerized Edeleanu extract and the like, thus leaving the so-called maltenes and the lighter coloured asphaltenes dissolved in the precipitating agent. The remaining, i. e. not precipitated, portion (further concentrated or not) of the polymerized extract may be referred to as the active portion of such extracts.

Before applying the above described refining treatment to the polymerized Edeleanu extract and the like, these materials may be concentrated by distilling off more volatile components (with steam or under vacuum, if desired, so as to avoid cracking at this stage) and/or reheated, thereby increasing the content of pour point-reducing components. The reheating can be done, for instance, at a mild cracking temperature, such as about 350° C.

The active pour point-reducing substances may be concentrated in the raffinate obtained by distilling off more volatile components from said raffinate substantially without causing the cracking of the resulting distillation residue. The raffinate may be further activated by reheating same substantially without distillation or cracking e. g. by prolonged heating at a temperature of about 350° C.

## Example

Edeleanu extract with a Saybolt-Furol viscosity of 36" at 25° C., derived from a spindle oil frac-

tion, was heated for 4 hours to 400° C. under a pressure of about 5 atmospheres. The polymerization product, which was obtained with a yield of 75%, was concentrated by steam distillation to 5 a residue of 15-20% calculated on the original extract; it had the appearance of a hard asphalt or pitch. This residue was mixed at about 100° C. with 2 volumes of kerosene containing about 8% aromatics. After being cooled, the solution was 10 decanted (it could be filtered) and the kerosene evaporated with steam. The resulting residue (6% of original extract) was the desired product which was used for reducing pour points of mineral oils.

15 When this product was added to three different lubricating oils with pour points 0° C., +1° C. and -6° C. in proportion of 1%, the pour points were reduced by 12, 10 and 9° C., respectively.

20 In order to obtain a liquid product, a suitable quantity of a lubricating oil can be added before evaporating the kerosene or other precipitant; the distillation (carried out at non-cracking temperatures) is so controlled then as not to distil 25 off the added lubricating oil, so that it remains in the residue and the final product (residue) is obtained in the liquid form.

Instead of a kerosene also a lubricating oil fraction poor in aromatics can be used as the 30 precipitating agent, such, for instance, as an Edeleanu raffinate, which may have been treated with an acid. After filtering or centrifuging the resulting product can be used directly as a pour point-reducing agent.

35 I claim as my invention:

1. In the process of lowering the pour point of a mineral oil, the steps of precipitating asphaltenes from a polymerized extract derived by extracting mineral oil with a selective solvent 40 for non-paraffinic hydrocarbons by adding a liquid precipitant for asphaltenes to said polymerized extract, removing the precipitate and the precipitant from the unprecipitated portion, thereby concentrating active pour point-reducing 45 substances in the unprecipitated portion, and adding the said concentrated pour point-reducing substances to the mineral oil.

2. The method of lowering the pour point of a viscous mineral oil, which comprises the step of 50 incorporating into said oil an effective quantity of a polymerized SO<sub>2</sub> soluble mineral oil extract rich in non-paraffinic hydrocarbons, substantially free from substances which are insoluble in light saturated aliphatic hydrocarbons.

55 3. In the process for preparing pour point reducing substances, the steps of adding a liquid precipitant for asphaltenes to a polymerized SO<sub>2</sub> soluble mineral oil extract rich in non-paraffinic hydrocarbons, thereby dissolving a portion of said 60 polymerized extract in the precipitant and precipitating asphaltenes from the dissolved portion, and separating the precipitate from the unprecipitated portion of the polymerized extract.

65 4. The process according to claim 3, in which the liquid precipitant is a light hydrocarbon rich in saturated aliphatic hydrocarbons.

5. The process according to claim 3, in which the liquid precipitant is a lubricating oil which is 70 poor in aromatics.

6. The process according to claim 3, in which the liquid precipitant is a mixture of alcohol and ether.

7. In the process for preparing pour point reducing substances, the steps of adding a liquid precipitant for asphaltenes to a polymerized SO<sub>2</sub> soluble mineral oil extract rich in non-paraffinic hydrocarbons, thereby dissolving a portion of said 5 polymerized extract in the precipitant and precipitating asphaltenes from the dissolved portion, separating the precipitate from the solution of precipitant and unprecipitated polymerized extract, separating the precipitant from the unprecipitated portion of the polymerized extract by distillation, and then distilling off the relatively 10 more volatile components of said unprecipitated portion substantially without causing the cracking of the resulting distillation residue, thereby 15 concentrating active pour point reducing substances in said residue.

8. In the process for preparing pour point reducing substances, the steps of adding a liquid precipitant for asphaltenes to a polymerized SO<sub>2</sub> soluble mineral oil extract rich in non-paraffinic hydrocarbons, thereby dissolving a portion of 20 said polymerized extract in the precipitant and precipitating asphaltenes from the dissolved portion, separating the precipitate from the solution 25 of the precipitant and unprecipitated portion of the polymerized extract, removing said precipitant from said solution by distillation, and activating the resulting unprecipitated portion of the polymerized extract by heating the same at 30 about 350° C.

9. In the process for preparing pour point reducing substances from a polymerized SO<sub>2</sub> soluble hydrocarbon oil extract containing the same, the steps of concentrating said polymerized extract rich in non-paraffinic hydrocarbons by distilling it to remove the relatively more volatile components, adding a liquid precipitant for asphaltenes to the resulting distillation residue, thereby dissolving a portion of said residue in 35 the precipitant and precipitating asphaltenes from the dissolved portion, and separating the precipitate from the unprecipitated portion of said distillation residue.

10. In the process for preparing pour point reducing substances, the steps of adding a hydrocarbon fraction which is poor in aromatic hydrocarbons to a pyrogenous polymerization product of an SO<sub>2</sub> soluble mineral oil extract rich in non-paraffinic hydrocarbons, thereby dissolving a portion of said polymerization product and precipitating asphaltenes, and removing the precipitate from the unprecipitated portion of the polymerization product.

11. As a new composition, a wax-bearing lubricating oil containing the asphaltene-free portion of a polymerized liquid sulfur dioxide soluble extract from mineral oil.

12. As a new composition, a wax-bearing lubricating oil containing that portion of polymerized SO<sub>2</sub> soluble mineral oil extract which is soluble in light saturated aliphatic hydrocarbons, and substantially free from substances which are insoluble in light, saturated aliphatic hydrocarbons.

13. As a new composition, a wax-bearing lubricating oil containing that portion of a pyrogenous condensation product of SO<sub>2</sub> soluble mineral oil extract which is soluble in light saturated aliphatic hydrocarbons, and substantially free from substances which are insoluble in light saturated aliphatic hydrocarbons.